

June 4, 1957

E. Q. SYLVESTER

2,794,224

METHOD OF COOLING CAST METAL PREFERENTIALLY

Filed June 8, 1953

2 Sheets-Sheet 1



Fig. 1.

INVENTOR.  
*Edmund Q. Sylvester*  
BY  
*Wm. O. Farmer*  
*Atty.*

June 4, 1957

E. Q. SYLVESTER

2,794,224

METHOD OF COOLING CAST METAL PREFERENTIALLY

Filed June 8, 1953

2 Sheets-Sheet 2



*Fig. 3.*



INVENTOR.  
*Edmund Q. Sylvester*  
BY  
*John O. Farmer*  
*Atty.*

1

2,794,224

## METHOD OF COOLING CAST METAL PREFERENTIALLY

Edmund Q. Sylvester, Chicago, Ill., assignor to Griffin Wheel Company, Chicago, Ill., a corporation of Delaware

Application June 8, 1953, Serial No. 359,997

6 Claims. (Cl. 22—212)

This invention relates to foundry practice and more particularly to a novel method and means for eliminating hot tears in castings of metal such as steel and other ferrous metals.

When molten metal such as steel is poured into a conventional mold, freezing or solidification of the metal is initiated by the formation of an envelope of solid metal at the mold and metal interface.

If the casting is of simple form, the envelope develops with substantially uniform thickness over the surface of the entire casting because the heat of the molten metal is uniformly dissipated and absorbed by the mold thereby preventing the development of hot tears.

According to the present invention, however, it has been discovered that the pouring of annular castings, such as wheels in graphite molds, although producing unusually fine castings at low cost, frequently results in hot tears because of the high heat conductivity of the graphite, a characteristic which is requisite in the production of castings suitable for use under conditions of severe wear and shock as, for example, railway car truck wheels.

In such molds a relatively thick envelope of solid metal is very rapidly formed throughout the entire surface of the casting with the exception of an area or areas fed by a riser or risers. Consequently, after the casting has solidified and the risers have performed their function of feeding the solidifying casting to prevent shrinkage cracks therein, solid contraction progressing through the entire casting tends to develop hot tears in the areas where the casting was connected to the risers.

According to the present invention, it has been discovered that the development of such hot tears can be eliminated without sacrificing other superior characteristics of such castings. This is accomplished by removing the risers after they have completed their function of feeding the solidifying casting and prior to solid contraction of the casting, and by subsequently cooling the riser sprues on the casting before such contraction takes place.

According to the invention, the cope and risers are removed immediately upon solidification of the casting. Thereafter, by means of a novel cooling apparatus, compressed air from a shop line at a pressure value of about 90 pounds per square inch is directed against the sprues where the risers were previously connected to the casting. This novel process affects an increase in the cooling rate of the metal beneath the surface of the sprues, so that the portions of the envelope in these areas become as thick and strong as the remainder of the surface of the casting prior to solid contraction thereof, whereby upon such contraction hot tearing is eliminated.

Other objects and advantages of the invention will become apparent from a consideration of the following specification and the accompanying drawings, wherein:

Figure 1 is a central vertical sectional view through a graphite mold and pressure pouring apparatus, prior to pouring of a casting;

Figure 2 is a fragmentary vertical sectional view simi-

2

lar to Figure 1 but showing the mold removed from the pouring apparatus with the mold cope and risers removed from the casting and showing the novel sprue cooling apparatus associated with the casting;

Figure 3 is a plan view of the sprue cooling apparatus shown in Figure 2;

Figure 4 is a side-elevational view of one of the sprue cooler units applied to the casting which is fragmentarily illustrated in cross section, and

Figure 5 is a bottom plan view of the sprue cooler unit shown in Figure 4.

Describing the invention in detail and referring first to Figure 1, a ladle 2 containing a body of molten metal, such as steel, is disposed in a pressure chamber 4 having a sealed cover 6 and having a conduit 8 for the passage of a pressure gas such as air.

The cover 6 is provided with an opening 10 within which a pouring tube 12 is sealed. The tube is provided at its upper end externally of the chamber 4 with a head 14 seated at the underside thereof on a tapered gasket 16 supported by the top of the cover 6. Thus the tube 12 and head 14 are maintained in tilted position, as described in detail and claimed in my copending application, Serial No. 299,071, filed July 16, 1952, now abandoned, for Casting Method and Apparatus.

The head 14 is provided with an upwardly tapering conical seat 18 adapted to mate with a complementary seat 20 defining the margin of an opening in the bottom of a tray or pan 22 containing a drag 24 of a graphite mold which also comprises a cope 26. The cope and drag may be formed of any suitable solid refractory material machined to define a casting cavity 28. However, the cope and drag 24 and 26 are preferably formed of graphite, the composition and the manufacture of which is set forth in detail in my copending application, Serial No. 189,961, filed October 13, 1950, for Wheel, Mold, and Method of Making.

The casting cavity 28 is connected by a gate 30 to the upper end of the tube 12, whereby upon admission of pressure gas to the chamber 4 through the conduit 8, the molten metal in the ladle 2 is forced upwardly through the tube 12 and gate 30 into the casting cavity 28 and upwardly therefrom into riser cavities 32, defined by baked sand cups 33 within complementary openings of the cope 26. Only one of the riser cavities is illustrated in Figure 1; however, it will be understood that preferably three, and if desired more, of such cavities may be equidistantly spaced from each other around the perimeter of the casting cavity 28, as described in detail in said copending application, Serial No. 189,961.

The cope 26 is also provided with a plunger 34 sleeved through a complementary opening of the cope and having a tapered head or seat 36 engageable with a complementary seat at the upper end of the gate 30 to seal the latter when the cavities 28 and 32 have been filled with molten metal, whereupon pressure in the chamber 4 is exhausted to accommodate removal of the graphite mold and assembling of another mold on top of the pouring tube 12, preparatory to pouring another casting.

Upon removal of the graphite mold from the pouring tube 12 and during a time interval of the order of about five minutes after pouring the metal in the mold freezes to form a casting 38 (Figure 2), which is fed during this period by risers of molten metal in the riser cavities 32.

At the end of this time interval the cope 26 is removed. Normally the risers break off and are removed with the cope; however, occasionally one or more of the risers and their associated cups 33 pull loose from the cope as the latter is lifted from the drag, and in this event such risers are immediately broken or cut off and are removed from the casting 38.

At this time the various sections of the casting are at

temperature values of from about 1800° F. to about 2300° F. and substantial solid radial contraction of the casting 38 has not yet taken place. Before substantial contraction does take place and while the sprues are at a temperature value of from about 2100° F. to about 2300° F., the novel sprue cooling apparatus 39 shown in Figures 2 to 5 is lowered into engagement with the rim of the casting which in the illustrated embodiment is in the form of a railway freight car wheel.

The sprue cooling apparatus 39 comprises three or more cooler units 40, the number of which corresponds to the number of risers utilized. Each unit 40 comprises a tank or chamber 42 connected to a pipe 44. The pipes 44 are in turn connected to a line 46 having a conventional shut off valve 48 as illustrated in Figure 2, said line 46 being connected to a supply of compressed gas such as compressed air from a shop line at a pressure of the order of about 90 pounds per square inch. The gas may be at or below room temperature.

The underside of each tank 42 is provided with a positioning lug or bracket 50 having converging positioning surfaces 52 and 54, as best seen in Figure 4. The surface 52 is adapted to seat on the upper edge of the rim of the casting 38, and the surface 54 is adapted to engage the outer perimeter or rim of the casting to properly position each unit 40 as shown in Figure 4, so that ports 56 of each chamber 42 direct compressed air against the related sprue 58 at a point where the casting 38 was fed during solidification thereof by one of the risers.

Compressed air is directed in this manner against the sprues 58 for a period of time of the order of approximately one minute to affect an increase in the cooling rate of the metal beneath the surface of the sprues 58 so that the envelope constituting the outer surface of the casting 38 is of substantially uniform strength throughout all portions of the casting, prior to solid contraction thereof, thereby eliminating hot tearing as the casting 38 contracts radially during cooling thereof to room temperature.

I claim:

1. A method of making a ferrous metal casting comprising pouring such metal when molten into a graphite mold having an annular casting cavity partly defined by a cope with a riser cavity communicating with said casting cavity, then after the metal has solidified in said mold to form a casting and a riser connected thereto, and before substantial solid contraction of said casting has occurred, removing the cope and disconnecting the riser from said casting, and then cooling an area on said casting where said riser has been disconnected from said casting, by directing a stream of compressed gas against said area while the remainder of said casting cools at room temperature, and finally terminating said stream of compressed gas and cooling the entire casting including said area at room temperature.

2. A method of making a metal casting comprising pouring such metal when molten into a mold having a casting cavity and having a riser cavity communicating with said casting cavity, then after the metal has solidified in said mold to form a casting and a riser connected thereto, and before substantial solid contraction of said casting has occurred, disassembling the mold and disconnecting the riser from said casting to form a rough area at

the point where said casting was connected to said riser; then before said contraction has occurred directing a stream of coolant gas against said area while cooling the rest of the casting at a room temperature, and finally terminating flow of said gas against said area and cooling the entire casting including said area at room temperature.

3. A method of making a casting comprising pouring molten metal into a mold having a casting cavity and having a riser cavity communicating with the casting cavity, then after the metal has solidified in said mold, to form a casting and a riser connected thereto, disassembling the mold and disconnecting the riser from said casting to form a spot on said casting at the point where said riser was connected thereto then cooling said spot at a rate substantially in excess of the cooling rate of the remaining surface area of the casting before substantial solid contraction of the casting has occurred, whereby such contraction does not produce a hot tear in the region of the sprue, and finally cooling the entire casting including said spot at room temperature until the entire casting is at room temperature.

4. A method of making a casting comprising pouring molten material into a mold having a casting cavity and a riser cavity connected thereto, then, after the material has solidified in said cavities, disassembling the mold and disconnecting the riser from the casting, and then before substantial solid contraction of the casting has occurred, directing a stream of compressed coolant gas against a spot on said casting at the point of interconnection between the riser and the casting, while cooling the remainder of said casting at room temperature, and finally terminating flow of said gas against said spot and cooling the entire casting including said spot at room temperature until the casting reaches room temperature.

5. A method of making a casting comprising pouring molten material into a mold having interconnected casting and riser cavities, then, after the material has solidified in said cavities, disconnecting the riser from the casting, and then before substantial solid contraction of the casting has occurred, cooling a spot on said casting formed by the connection thereof to said riser at a rate greater than the cooling rate of the remainder of said casting.

6. Apparatus for cooling hot spots in a wheel casting comprising a plurality of spaced heads, each of which comprises a plurality of ports for directing a coolant gas against its related spot, a surface on each head facing the ports thereof and formed and arranged to engage the tread surface of the wheel casting to position the apparatus relative thereto.

#### References Cited in the file of this patent

#### UNITED STATES PATENTS

|    |           |          |               |
|----|-----------|----------|---------------|
| 55 | 7,515     | Truscott | July 16, 1856 |
|    | 15,109    | Allen    | June 10, 1856 |
|    | 1,281,946 | Griffin  | Oct. 15, 1918 |
|    | 1,969,840 | Goddard  | Aug. 14, 1934 |
| 60 | 2,032,738 | Cramer   | Mar. 3, 1936  |
|    | 2,117,948 | Flammang | May 17, 1938  |

#### FOREIGN PATENTS

|         |        |               |
|---------|--------|---------------|
| 514,598 | France | Nov. 17, 1920 |
|---------|--------|---------------|